

# United States Patent

[19]

Nakajima et al.

[11] 3,912,515

[45] Oct. 14, 1975

[54] **SILVER HALIDE PHOTOSENSITIVE MATERIAL**

[75] Inventors: Tomio Nakajima; Masashi Nakano; Takashi Uchida; Ken-ichi Kishi, all of Tokyo, Japan

[73] Assignee: Konishiroku Photo Industry Co., Ltd., Tokyo, Japan

[22] Filed: Dec. 19, 1973

[21] Appl. No.: 425,977

[30] **Foreign Application Priority Data**

Dec. 28, 1972 Japan..... 47-130258

[52] **U.S. Cl.**..... 96/84 R; 96/84 UV; 96/88; 96/100

[51] **Int. Cl.<sup>2</sup>**..... G03C 1/84; G03C 1/40

[58] **Field of Search**..... 96/100, 84 UV

[56] **References Cited**

UNITED STATES PATENTS

3,658,546 4/1972 Doorselaer et al. .... 96/100  
3,676,142 7/1972 Carpentier et al. .... 96/100  
3,752,672 8/1973 DePauw et al. .... 96/100

3,788,857 1/1974 VanPoucke et al. .... 96/100

*Primary Examiner*—Ronald H. Smith  
*Attorney, Agent, or Firm*—Bierman & Bierman

[57] **ABSTRACT**

An improved silver halide photosensitive material is disclosed which comprises, as a high boiling point solvent for photographic additives such as couplers, at least one solvent selected from (1) straight or cyclic alkanes having at least 9 carbon atoms, (2) straight or cyclic alkenes having at least 9 carbon atoms, and (3) compounds represented by the following general formula:



wherein R<sub>1</sub>, R<sub>2</sub> and R<sub>3</sub> are individually hydrogen, alkyl, cycloalkyl or aryloxy, or R<sub>1</sub> and R<sub>2</sub> can cooperatively form a hydrocarbon ring as members thereof.

**3 Claims, No Drawings**

## SILVER HALIDE PHOTOSENSITIVE MATERIAL

This invention relates to a photographic material characterized in that a photographic additive which is usually added to a photographic material in the form dissolved in a high boiling point solvent, such as a ultraviolet absorber, a coupler and the like, is incorporated in a photographic material with use of a novel photographic solvent.

As is well known in the art, ultraviolet absorbers of the benzophenone type, the benztriazole type, the acrylonitrile type, the triazine type, and of the cyanomethylenebenzodithiol type are employed as photographic ultraviolet absorbers, and N-(2,4-di-tert-  
amylphenoxybutyl)-1-hydroxy-2-naphthamide of the following formula



1-(2,4,6-trichlorophenyl)-3-(2,4-di-tert-  
amylphenoxy)acetamido benzamido-5-pyrazolone of  
the following formula



and the like are employed for protected couplers. These additives are usually added to a photographic material in the state dissolved in a high boiling point solvent such as di-n-butyl phthalate, triphenyl phosphate, tri-o-cresyl phosphate, monophenyl-di-p-tert-butyl phosphate, monophenyl di-o-chlorophenyl phosphate, tri-p-tert-butylphenyl phosphate, di-p-tert-butylphenyl-mono-(5-tert-butyl-2-phenyl-phenyl) phosphate and the like.

However, these high boiling point solvents are still insufficient in the dissolving power.

For example, because of the insufficient dissolving power, the photographic additive is precipitated in the form of crystals at the step of coating a gelatin layer, and the presence of crystals of the photographic additive have bad influences on the properties of the coated photographic emulsion layer.

This invention is to provide a photographic material of good quality formed with use of a high boiling point solvent free of such defects involved in conventional high boiling point solvents.

The high boiling point solvent to be used in this invention is at least one member selected from the group

consisting of (1) compounds represented by the general formula



(wherein R<sub>1</sub>, R<sub>2</sub> and R<sub>3</sub> are respectively a hydrogen atom, alkyl, cycloalkyl, aryloxy, or R<sub>1</sub> and R<sub>2</sub> may form together a hydrocarbon ring,) (2) straight and cyclic alkanes having at least 9 carbon atoms and (3) straight and cyclic alkenes having at least 9 carbon atoms. These high boiling point solvents may be used singly or in the form of a mixture of two or more of them. It is also possible to employ these high boiling point solvents in combination with low boiling point solvents as in the case of conventional high boiling point solvents.

Typical instances of the high boiling point solvent to be used in this invention include cumene, p-cymene, mesitylene, di-isopropyl benzene, n-butyl benzene, sec-butyl benzene, t-butyl benzene, hexyl benzene, cyclohexyl benzene, dodecyl benzene, diphenyl ether, n-decane, decalin, tetralin, 1-dodecene, 1-decene, and 1-nonene.

Results of the test of the dissolving power of the solvents made with use of a ultraviolet absorber as the additive to be dissolved are shown below.

## TEST EXAMPLE

A mixture of four ultraviolet absorbers, 2-(2'-hydroxy-5'-tert-butylphenyl)benztriazole, 2-(2'-hydroxy-3'-tert-butyl-5'-di-tert-butylphenyl)benztriazole and 2-(2'-hydroxy-3', 5'-di-tert-butylphenyl)-5-chlorobenztriazole was used as the ultraviolet absorber. 1g of the above mixture was dissolved in 2ml of ethyl acetate and 1 ml of a high boiling point solvent indicated below in Table 1, and 20 ml of water was added to the solution.

The mixture was shaken and allowed to stand still. The time as which the ultraviolet absorber was precipitated was measured to obtain results shown in Table 1.

Table 1

|    |                     |                   | Time at Which Precipitation Of Ultraviolet Absorber Began |
|----|---------------------|-------------------|-----------------------------------------------------------|
| 50 | Comparative Solvent | dibutyl phthalate | within 3 hours                                            |
|    | Solvent of          | decalin           | more than 169 hours                                       |
| 55 | This invention      |                   |                                                           |
|    | "                   | 1-dodecene        | more than 168 hours                                       |
|    | "                   | isopropyl benzene | more than 168 hours                                       |
|    | "                   | n-dodecane        | more than 168 hours                                       |

As is seen from the results shown in Table 1, the solvent to be used in this invention has a much higher dissolving power than the comparative solvent. Therefore, when a ultraviolet absorber is added to elemental substances of a photosensitive material in the form dissolved in the solvent of this invention, defects in conventional solvents as above mentioned are eliminated.

Further, when a protected coupler is added to elemental substances of a photographic material with use

of the solvent of this invention, there can be obtained an excellent photographic material in which photographic properties are not damaged for a long period of time.

The solvent to be used in this invention is photographically harmless and has no bad influences on other photographic additives.

This invention will now be illustrated more detailedly by reference to examples.

#### EXAMPLE 1

A photosensitive silver chlorobromide gelatin emulsion for red sensitive containing a cyan coupler was coated on a raw paper for photographic use, and a gelatin solution containing a solution of the same ultraviolet absorber as used in Test Example which was prepared with use of a high boiling point solvent indicated in Table 2 was coated on the emulsion layer so that a protective gelatin layer was formed at a base weight of 6.0 mg/10 cm<sup>2</sup>. Then, the coated gelatin layer was dried to obtain a test sample.

The solution for formation of the gelatin protective layer was prepared by dissolving 3 g of the ultraviolet absorber in 6 ml of ethyl acetate and 3 ml of the high boiling point solvent, adding the solution to 60 ml of a 10% aqueous solution of gelatin containing saponin, emulsifying and dispersing the mixed solution by means of a colloid mill and adding 40 ml of water to the dispersed solution.

The so obtained sample was exposed to light, subjected to color development, hardening fixation, bleaching fixation and water washing, and then dried.

With respect to each sample, the red density of the cyan image and stain density (determined based on the blue color concentration) at non-image areas were measured. Then, the sample was exposed directly to sun-light for 55 hours while employing a blue scale as a comparison, and the red density and stain density were measured again. Results of the reduction ratio of the red density and the stain density are shown in Table 2.

Table 2

| Reduction Ratio of Red Color Density (density after sun light exposure concentration just after preparation of sample, %) | Stain Density             |                          | 55   |
|---------------------------------------------------------------------------------------------------------------------------|---------------------------|--------------------------|------|
|                                                                                                                           | before sun light exposure | after sun light exposure |      |
| blank (no ultra violet absorber)                                                                                          | 64                        | 0.03                     | 0.15 |
| dibutyl-phthalate                                                                                                         | 11                        | 0.03                     | 0.06 |
| decalin                                                                                                                   | 10                        | 0.03                     | 0.06 |
| 1-dodecene                                                                                                                | 10                        | 0.03                     | 0.06 |
| isopropyl benzen                                                                                                          | 11                        | 0.03                     | 0.07 |
| n-dodecane                                                                                                                | 11                        | 0.03                     | 0.06 |
|                                                                                                                           |                           |                          | 60   |

As is seen from the results shown in Table 1, the protective gelatin layer containing a solvent according to this invention exhibits fading preventive effect and stain preventive effect substantially equal to these of a gelatin protective layer containing a solvent of dibutyl phthalate.

On the other hand, the solution comprising photographic additives and the solvent according to this invention exhibited more stability than the solution comprising photographic additives and the dibutyl phthalate, that is, crystallization did not occur on and before coating at all. When as ultraviolet absorber, 4,7-bis(β-ethoxyethoxy)-2-dicyanomethylene-1,3-benzodithiole was used instead of a mixture of four kinds of benztriazole, supreme results are also obtained as same as the above.

#### EXAMPLE 2

20 mg of 1-(2,4,6-trichlorophenyl)-3-[3-{(2,4-di-tert-amylphenoxy)-acetamide}-benzamide]-5-pyrazolone was dissolved in 20 ml of 1-nonenone and 60 ml of ethyl acetate (maintained at 60°C), and the solution was mixed with 10 ml of a 10% aqueous solution of Alkanol B and 200 m of a 5% aqueous solution of gelatin. The mixture was emulsified and dispersed by means of a colloid mill.

The so obtained dispersion was added to 1 Kg of a silver chlorobromide emulsion for formation of photographic papers, and the mixture was coated on a raw papers, and dried. The so obtained sample was exposed to green light exposure, subjected to color development hardening fixation, bleaching fixation and water washing, and dried. As a result, there was obtained an image of a magenta color comparable to the image obtained by employing dibutyl phthalate instead of 1-nonenone.

What is claimed is:

1. In a silver halide photosensitive material comprising a high boiling point solvent for photographic additives, the improvement which comprises said solvent being selected from a group consisting of straight or cyclic, alkanes and alkenes having at least 9 carbon atoms; and cumene, p-cymene, mesitylene, di-isopropyl benzene, n-butyl benzene, sec-butyl benzene, t-butyl benzene, hexyl benzene, cyclohexyl benzene, dodecyl benzene and dephenyl ether.

2. A silver halide photosensitive material according to claim 1 wherein said photographic additives are couplers.

3. A silver halide photosensitive material according to claim 1 wherein said photographic additives are ultraviolet absorbers.

\* \* \* \* \*